# EUROPEAN PATENT SPECIFICATION

(11) **EP 2 530 189 B1**
(45) Date of publication and mention of the grant of the patent: **13.06.2018**
(21) Application number: 12168226.4
(22) Date of filing: 16.05.2012
(51) Int. Cl.: D01F 11/00, D01D 5/00, D06M 23/08, B32B 5/26

(54) **Method of production of functional nanofiber layer and device for carrying out the method**
Verfahren zur Herstellung von funktionellen Nanofaserschichten sowie Vorrichtung zur Ausführung des Verfahrens
Procédé pour la production de couches de nanofibres fonctionelles et appareil pour appliquer ce procédé

(30) Priority: 01.06.2011 CZ 20110328
(43) Date of publication of application: 05.12.2012
(73) Proprietor: Technicka Univerzita V Liberci, 461 17 Liberec 1 (CZ)
(72) Inventor: Pokorný, Pavel, 46401 Frýdlant v Cechách (CZ); Louda, Petr, 46341 Dlouhý most (CZ); Lukás, David, 46006 Liberec (CZ); Mikes, Petr, 46331 Mnísek u Liberce (CZ); Vyslouzilová, Lucie, 79811 Prostejov (CZ); Chvojka, Jirí, 46001 Liberec (CZ); Hégrová, Bozena, 46001 Liberec (CZ); Lukás, Richard, 46322 Mnísek u Liberce (CZ); Amler, Evzen, 17000 Praha (CZ); Buzgo, Matej, Turna nad Bodvou (SK)
(74) Representative: Musil, Dobroslav

(56) References cited:
- EP-A1- 1 264 804
- CN-A- 101 947 415
- JP-A- 2008 285 793
- KR-A- 20070 097 936
- US-A1- 2003 069 369
- THOPPEY N M ET AL: "Unconfined fluid electrospun into high quality nanofibers from a plate edge", POLYMER, ELSEVIER SCIENCE PUBLISHERS B.V, GB, vol. 51, no. 21, 1 October 2010 (2010-10-01), pages 4928-4936, XP027321065, ISSN: 0032-3861 [retrieved on 2010-08-14]

## Description

### Technical field

A method for producing a functional nanofiber layer comprising particles of solid and liquid matter by means of electrospinning of a solution or melt of a polymer, at which the produced nanofibers are laid up between a spinning electrode and a collecting electrode onto a base which is the surface of the collecting electrode or a carrying material.

A device for producing a functional nanofiber layer comprising particles of a solid or liquid matter by means of electrospinning of a solution or melt of a polymer between a spinning electrode and a collecting electrode, at which the nanofibers being produced are laid up between the spinning electrode and the collecting electrode onto a base which is the surface of the collecting electrode or a carrying material.

### Background art

The production of nanofibrous layers is usually carried out by means of electrospinning or other well-known methods (usually by means of melt-blowing, drawing or centrifugation). Thereat, small particles are brought into a polymer solution or melt, where they are dispersed. Subsequently, the substance being obtained that way is spun. The second method is based on utilizing the so called coaxial electrospinning. Thereat, a material gets incorporated into the fiber cores, which does not need to be spinnable itself. Among others, liquid dispersions of particles of a solid matter or globules of liquid of a suitable size can be used for the purpose.

The objective of such solutions is the production of nanofibers obtaining the requested qualities by the incorporation of given particles. By means of subsequent leaching, the material of the particles can also be removed from the fibers, porous fibers with nano-cavities occurring after the material has been washed out being obtained.

CN 101586256 A solves a method for the production of porous electrospun fibers with nano-salt equally dispersed in a polymer solution, a component fiber (polymer + nano salt) being obtained by means of electrospinning. By means of subsequent leaching of the saline solution the salt is separated, openings are created and the final porous fiber is produced.

Biologically activated carbon fiber for medical purposes and its production is proposed by CN 101736441 A. Electrospinning and high-temperature sintering is carried out to obtain nanoparticles of calcium phosphate with biological activity in the carbon fibers. The diameter of the carbon fibers varies from 50 to 500 nm; the size of nanometric particles of calcium phosphate varies from 10 to 100 nm; the percentage by weight is between 1 and 10 %. Dispersed nanoparticles of calcium phosphate strengthen the bio-bond between the carbon nanofiber and the bone tissue and usually improve the ability of induced bone development.

The objective of KR 20090058155 A is the production of antibacteriological, aseptic and at the same time biologically degradable wrapping paper as a means for filtering air or water. The paper is highly temperature-resistant and mechanically strong. It is made of nanofibers produced by means of electrospinning of a solution having antibacteriological and antiseptic qualities. It contains metallic particles and biodegradable fiber-forming polymer.

A part of the WO 2008077372 file deals with the method and device for the production of composite fibrous material. At first, fibers of non-ionic polymer are sulphonated. Sulphonated, and thus anionically behaving fibers mix with a polyamide solution in the next step, to make their behaviour cation-active. Finally, the fibers are brought into contact with an anionic dispersion of particles, by means of which the particles get bound to the surface area of the fibers and a fiber-particle composite is produced.

CZ 300797 B6 relates to a textile comprising at least one layer of polymeric nanofibers obtained by electrospinning from a polymer solution, the polymeric nanofibers comprising particles of a low-molecular matter. The nanofibers of the low-molecular matter are products of a chemical reaction of the low-molecular matter antecedent dissolved in a polymeric solution and a chemical agent applied onto the nanofibers after their spinning. The polymer solution for spinning contains a low-molecular matter antecedent. At spinning, the low-molecular matter antecedent together with the polymer are pulled into the nanofibers being produced. After spinning, a suitable chemical agent is used to act on the antecedent contained in the nanofibers, by means of which the low-molecular matter antecedent transforms into a low-molecular matter.

CZ 297774 B6 solves the method of the production of photocatalytically active TiO₂. The production starts from a very cheap raw material - alkaline titanate, which is the by-product of the production of titanium white. The titanate is acted upon by glycol while being heated up and the mixture is then processed by sulphuric acid. The product is photocatalitically active TiO₂ of nanofibrous morphology.

According to CZ 300805 B6, a bio-material based on nanofibrous layers consists of at least two nanofibrous layers, covered by living cells growing on their both sides interconnecting those layers. The nanofibrous layers are unwoven and are composed of synthetic polymers or copolymers of monomers selected from a group comprising methacrylic acid esters, methacrylic acid amides, urethanes, vinyl alcohol and monomers derived from lactic acid and its derivatives, and the method of its preparation. At spinning, the cells are sown on an unwoven layer of nanofibers.

CZ 2008-241 A3 makes a wrapping agent public, which is namely a wrapping agent comprising woven or unwoven textile comprising nanofibers and evaporative corrosion inhibitors.

CZ20096-148 makes an electrospinning device public, containing two serial separated spinning apparatuses. The first of them generates a supporting layer of nanofibers, microfibers and/or liquid nanoparticles containing polyisobutylene on the carrying material. The second spinning device lays the actual functional layer of nanofibers onto the base. The double device is expensive, actually solving only the perfection of the bond of certain functional nanofiber layers to the carrying material and having only an indirect influence on the qualities of the functional nanofiber layer.

The methods and devices according to the prior art are particularly complicated, not dealing with continuous manufacturing of the final composite product, which in the case is a system of nanofibers with particle material invested. Moreover, the quality of the products depends on the required synchronization of the individual steps of its production. The objective of the invention is to relieve the shortages of the prior art or to reduce them to a significant extent and to propose a reasonably priced method of production of a nanofibrous layer allowing to influence its functional qualities by means of adding powdery particle material.

### Principle of the invention

The objective of the invention is achieved by means of a method for producing a functional nanofibrous layer comprising particles of either a solid or a liquid matter, the goal of which is that particles are brought into the nanofibrous layer by joint action of gravitational forces, when the particles are guided along an inclined skid plate ended with a sharp edge, and the action of high voltage between a base and the particles which by contacting the charged edge of the skid plate acquire an electric charge consistent with the charged edge, whereby at the same time, ionization of the gaseous environment occurs and electric wind is formed, leading away from the sharp edge of the skid plate, which helps with the transport of the particles being incorporated to the surface area of the collecting electrode. The movement of the particles on the inclined skid plate is facilitated by vibrations of the skid plate.

The objective of the invention is also achieved by means of a device for the production of a functional nanofibrous layer comprising solid or liquid matter particles, in which at least one tank with an outlet opening for batching the solid or liquid matter particles is arranged behind the place and/or in the place of deposition of the nanofibers towards the base, the principle of which is that the outlet opening of the tank is coupled with a skid plate equipped with a sharp edge at its end facing the base, the skid plate is connected to a high voltage power supply. That allows to produce a narrow current of electric wind directed away from the sharp edge, which facilitates the transport of suitably sized particles into the wind current and further to the desired place.

The skid plate is connected to an outlet member of a vibrator, whose vibrations facilitate the transport of the solid particles.

From the point of view of the surface requirements of the emerging product and the production of a compact layered band, it is advantageous to place a spinning electrode behind the place of deposition of the particles being brought in.

### Description of the drawing

The device is schematically represented in the drawing, where Fig. 1 shows a device according to Background art, Fig. 2 shows a design comprising two particle tanks, Fig. 3 shows a device according to the invention using the combined effect of gravity, vibrations electric wind and Coulomb forces to incorporate the particles, Figs. 4 and 5 show a device according to background art using the effect of an electrospraying system to incorporate the particles and a continuously operating device processing two types of nanofibers and two types of incorporated particles.

### Examples of embodiment

An exemplary embodiment of the device according to background art for incorporating solid or liquid matter particles into a nanofibrous layer at electrospinning comprises a spinning electrode **1** equipped with an output nozzle **11** for importing the processed polymer into an electic field between a spinning electrode **1** connected to the positive pole **10** of a high voltage power supply and a collecting electrode **2** comprising a rotating collector connected to the negative pole **20** of a high voltage power supply. The cylindrical or other surface of the collecting electrode **2** is either covered in a non-represented carrying material or makes up a surface onto which the nanofibers are laid up directly, being removed after finishing the production of the respective layer. Above the collecting electrode **2** a tank **3** is placed, being filled with fine particles of material, which are meant to be incorporated into the final composite nanofibrous material. In the exemplary embodiment, the tank **3** is advantageously connected to the positive pole **10** of the high voltage power supply. In a different embodiment, the tank **3** can be gravitational. In an advantageous embodiment, the tank is coupled with a non-represented vibrational device. The tank **3** is equipped with a lockable outlet **31.**

The device represented in Fig. 2 is supplemented by another tank **4** for particles having qualities different from those deposited in tank **3.**

In Fig. 3, a tank **5** for particles is placed, the lower part of which is connected to a bottom comprising a skid plate **6,** having a sharp edge **61** neighbouring the collecting electrode **2** and the outlet nozzle **11** of the spinning electrode **1.** The edge **61** is connected to the positive pole of the power supply. The wall of the tank **5** is finishes in a lockable outlet **51** in its lowest place. In an advantageous embodiment, the skid plate **6** is connected to an outlet member of a non-represented vibrator.

In Fig. 4 the device according to the background art is represented, the tank for particles of which is made up of an electrospraying system **7** with a reservoir **71** for the spraying liquid, the outlet tube **72** of which is brought close to the collecting electrode **2** and the outlet nozzle **11** of the spinning electrode **1.** The electrospraying nozzle **73** is directed into the area of the collecting electrode **2,** onto which the nozzle **11** of the spinning electrode **1** is directed as well. The outlet tube **72** is connected to the positive pole **10** of the high voltage power supply. In a non-represented embodiment, there is a tank for solid particles instead of a reservoir **71** for the spraying liquid.

In a non-represented embodiment, there are devices included, comprising electrical means for the atomization of particles and their transport towards the surface of the collecting electrode, which are represented in Fig. 3 and 4, is supplemented by supportive pneumatic means. Those comprise a compressed air feeding pipeline the outlet nozzle of which neighbours the outlet opening **51** of the tank **5** of particles or the outlet tube **72** orifice directed towards the surface of the collecting electrode **2.**

In Fig. 5, a device according to the invention is represented, intended for a continuous production of a nanofibrous layer with incorporated particles. In contrast to the embodiment according to Fig. 1 to 4, a part of the collecting electrode **2** is belted with a band of carrying material **8,** led by a pair **81** of intake rollers before the collecting electrode **2** and by a pair **82** of off-take rollers after the collecting electrode **2.** In the vicinity of the part of the collecting electrode **2** circuit opposite to the spinning electrode **1** another spinning electrode **12** is placed.

In Fig. 6, another embodiment of the device according to the background art is represented, intended for a continuous production of a nanofibrous layer with incorporated particles. The motion of the carrying material **8** band in the **S1** direction is mediated by means of a pair **83** of feed rollers and a pair **84** of detaching rollers. In the spinning chamber **9,** the spinning electrode **1,** the tank **4** for particles, the spinning electrode **12** and the tank **4** for particles are placed gradually in the **S1** direction of the carrying material **8** band's motion above the carrying material 8. Below the band of carrying material **8,** two collecting electrodes **13** are placed under the spinning electrodes **1, 10** and two collecting electrodes **14** are placed under the tanks **3, 4.** In a non-represented embodiment, two spinning electrodes **1, 12** are placed in a row, having tanks **4** and **3** for particles in a row after them.

A layer of nanofibers distributed in a commonly known way (Fig. 1), comes under the outlet opening **31** of the tank **3** for particles after the collector **2** has been turned in the **S2** direction. After the outlet opening **31** has been opened, the particles are poured into a layer of nanofibers by means of gravitation and/or the effect of the voltage difference occurring between the tank **3** for particles and the collecting electrode **2.** Thereat, the collecting electrode **2** can perform several revolutions when producing a single fibrous film, whereupon sandwich material gets produced, in the layers of nanofibers of which the poured particles are incorporated in the gaps between the nanofibers.

With the device according to Fig. 2, two kinds of particles from tanks **4** and **3** get gradually laid up after the distribution of the nanofibers.

In the exemplary embodiment according to Fig. 3, the tank **5** for particles is placed as close as possible to the spinning electrode **1** or its outlet nozzle **11.** After the outlet opening **51** of the tank **5** has been opened to pour the particles, the particles lying directly on the skid plate **6** are moved through the outlet opening **51** towards the edge **61** of the skid plate **6.** Such movement of particles may be facilitated by vibrations of the skid plate **6.** The sharp edge **61** connected to the positive pole **10** of the efficient high voltage power supply charges the powdery particles electrically. Ionization of the gaseous environment occurs and electric wind is formed. The current of electric wind in the **S3** direction away from the edge **61** is very narrow (forming a so called stream); that is why quick flux occurs in the vicinity of it, helping transport suitably sized particles into the current and further to a required place, i.e. to the surface area of the collecting electrode **2** virtually simultaneously with the stream of nanofibers leaving the outlet nozzle **11** of the spinning electrode **1.** Hereat, the like electric charge obtained by the particles contacting the charged edge **61** is utilized. The like charged particles then repel each other and obstruct the bunching of minute particles. At the same time, those charged particles are gravitated towards the collecting electrode by Coulomb forces, which also supports their motion.

The electrospraying system according to Fig. 4 uses a strong electric field to transport the particles. By means of it, the surface level of the spraying liquid transported through the outlet tube **72** from the reservoir **71** for the spraying liquid gets unbalanced, whereupon small droplets occur through so called electrospraying. Those droplets occurring after a contact with the charged edge of the nozzle **73** of the outlet tube **72** get seized by the current of the electric wind and transported to a required place. In this case, that is straight into the area where the fibers making up the nanofibrous layer are laid up simultaneously. The composite nanofibrous material is simultaneously produced in one place of the base material.

After using the atomizing device according to the invention, it is not necessarily needed to use the oppositely charged counter-electrode as the potential of the charged edge forming the electric wind is related to the ground consisting in e.g. the frame of the machine, the floor of the room etc.

An analogical electrospraying system may also be using already existing particular materials sputtered electrostatically onto the surface of the collecting electrode virtually simultaneously with the nanofibers.

With the non-represented devices described above, electric forces and aerodynamic effects of the air current lead from the respective source of compressed air are used for transporting the particles to the surface of the collecting electrode or for atomizing the liquid. The compressed air is used to support the effects of the electric field or, with devices not utilizing the electric field to transport particles, the aerodynamic effect of the compressed air is the only driving agent of the particles distributed into the nanofibrous layer.

Methods commonly known so far can also be used for the transport of particles and their batching. With one of those, the particles are transported by means of rotating or otherwise moving brushes. A device utilized with another commonly known method, comprises a surface-structured rotating roller, carrying the particles in cavities made on its surface and pouring them into the nanofibrous layer being formed.

The embodiments represented in Fig. 1 to 4 and their modifications related to the mutual arrangement of the spinning electrodes and tanks for particles allow to produce extensive sandwich material of a required thickness, which may comprise layers of nanofibers of different kinds, by means of multiple rotations of the collecting electrode **2** in the **S2** direction.

The collecting electrode **2** of the device according to Fig. 5 is partly banded with a carrying material **8** band. Its continuous motion in the **S4** direction is derived from the rotation of the collecting electrode **2** in the **S2** direction or the interaction of the pair **81** of the input rollers and the pair **82** of the off-take rollers, which are linked to non-represented driving means. In the exemplary embodiment, a layer of nanofibers produced by the spinning electrode **1** is primarily produced, followed by the particles from tanks **4, 3** being gradually incorporated into that layer and overlayed by a layer of nanofibers produced by the spinning electrode **12** afterwards. The band of carrying material **8** covered in a multicomponent nanofibrous layer is taken off by means of a pair **82** of off-take rollers for storing purposes or further processing.

With the device for continuous production of nanofibrous material, represented in Fig. 6, a band of carrying material **8** is lead through a lengthwise arranged spinning chamber **9** virtually horizontally in the **S1** direction, being driven by means of a pair **83** of feed rollers supported by a pair **84** of detaching rollers. After the band of carrying material **8** has entered the spinning chamber **9** the first nanofibrous layer, the first kind of particles, the second nanofibrous layer and the second kind of particles are gradually distributed onto it. The produced multicomponent nanofibrous material is detached from the spinning chamber **9** by means of a pair **84** of detaching rollers. The resulting multicomponent nanofibrous material can be modified through changing the order of spinning electrodes **1, 12** and tanks **4, 3.** That way, a second layer of nanofibers produced by means of spinning electrode **12** can be added to the first layer of nanofibers produced by means of spinning electrode **1** and the first kind of particles from tank **4** and subsequently the second kind of particles from tank **3** can be poured.

The represented and described embodiments according to the invention are not of a limiting effect. Their arrangements and modes of operation can be modified within the range of the patent claims, e.g. in terms of the direction of the nanofibers being fed in relation to the motion of the base which they are distributed on. The places where incorporated particles get bound to the nanofibrous layer can change similarly. Different kinds of particles can, for instance, be brought into virtually the same place of the nanofibrous layer based on current needs.

### List of reference marks

- 1: spinning electrode
- 10: positive pole (of the HV power supply)
- 11: outlet nozzle (of the spinning electrode)
- 12: spinning electrode
- 13: collecting electrode
- 14: collecting electrode
- 2: collecting electrode
- 20: negative pole (of the HV power supply)
- 3: tank
- 31: outlet opening (of the tank)
- 4: tank
- 5: tank (including the skid plate)
- 51: outlet opening (of the tank with the skid plate)
- 6: skid plate
- 61: edge (of the skid plate)
- 7: electrospraying system
- 71: reservoir (for the spraying liquid)
- 72: outlet tube (of the spraying liquid)
- 73: electrospraying system
- 8: carrying material
- 81: pair of input rollers
- 82: pair of off-take rollers
- 83: pair of feed rollers
- 84: pair of detaching rollers
- 9: spinning chamber
- S1: direction of the carrying band motion (in chamber 9)
- S2: direction of the rotation of the collector
- S3: direction of the electric wind streaming
- S4: direction of the carrying band motion

## Claims

1. A method for producing functional nanofibrous layers comprising particles of a solid or liquid matter by means of electrospinning of a solution or a melt of a polymer, with which the produced nanofibers are laid up between the spinning electrode (1) and the collecting electrode (2) onto a base, which is the surface of the collecting electrode (2) or a carrying material (8), whereby into thus formed layer immediately after its formation particles of the solid or liquid matter are brought between the nanofibers of the layer in the direction towards the base, whereby the particles are deposited in the gaps between the nanofibers, **characterized in that** the bringing of the particles into the nanofibrous layer is performed by the joint action of gravitational forces, when the particles are guided along an inclined skid plate (6) ended with a sharp edge (61) and by the action of high voltage between the base and the particles which in contact with the charged edge of the skid plate acquire an electric charge consistent with the charged edge (61), whereby at the same time, ionization of the gaseous environment occurs and electric wind is formed, leading away from the sharp edge (61) of the skid plate (6), which facilitates the transport of the particles being incorporated to the surface area of the collecting electrode (2).

2. The method according to claim, **characterized in that** the movement of the particles on the skid plate (6) is facilitated by vibrations of the skid plate (6).

3. A device for producing a functional nanofibrous layer comprising particles of a solid or liquid matter by means of electrospinning of a solution or melt of a polymer between a spinning electrode (1) and a collecting electrode (2), with which the produced nanofibers are laid up between the spinning electrode (1) and the collecting electrode (2) onto a base which is the surface of the collecting electrode (2) or a carrying material (8), whereby directly after the place and/or at the place of laying up the nanofibers there is placed opposite the base at least one tank (5) with an outlet opening (51) for batching the particles of the solid or liquid matter, **characterized in that** the outlet opening (51) of the tank (5) is coupled with the skid plate (6) equipped with a sharp edge (61) at its end neighbouring the base, whereas the skid plate (6) is connected to a high voltage power supply.

4. A device according to claim 3, **characterized in that** the skid plate (6) is connected to an outlet member of a vibrator

5. The device according to claim 3 or 4, **characterized in that** a spinning electrode (1, 12) is arranged after the place for depositing the particles being brought in.

## Patentansprüche

1. Verfahren zur Erzeugung einer Funktionsnanoschicht, die die Partikel eines festen oder flüssigen Stoffes durch elektrisches Verspinnen der Polymerlösung oder -schmelze aufweist, bei dem die gebildeten Nanofasern zwischen der Spinnelektrode (1) und der Sammelelektrode (2) auf eine Unterlage gelagert werden, die die Oberfläche der Sammelelektrode (2) oder ein tragendes Material (8) ist, wobei in so gebildete Schicht unmittelbar nach deren Erzeugung in der Richtung gegen die Unterlage zwischen ihre Nanofasern die Partikel eines festen oder flüssigen Stoffes eingetragen werden, die in den Spalten zwischen den Nanofasern gelagert werden, **dadurch gekennzeichnet, dass** die Eintragung von Partikeln in die Nanofaserschicht durch gemeinsame Schwerkraftwirkung, wann die Partikel auf einer geneigten Gleitplatte (6) geführt werden, die mit einer scharfen Kante (61) beendet ist, und durch die Wirkung der Hochspannung zwischen der Unterlage und den Partikeln erfolgt, die im Kontakt mit der geladenen Kante (61) der Gleitplatte (6) elektrische mit der geladenen Kante (61) übereinstimmende Aufladung erhalten, wobei es zugleich zur Ionisierung des gasförmigen Umfeldes und zur Entstehung der elektrischen Luft kommt, die von der scharfen Kante (61) der Gleitplatte (6) gerichtet ist, was dem Transport des eingetragenen Partikels zur Oberfläche der Sammelelektrode (2) beiträgt.

2. Verfahren nach dem Anspruch 1, **dadurch gekennzeichnet, dass** die Bewegung der Partikel auf der geneigten Gleitplatte (6) durch die Vibrationen dieser Rutschplatte (6) unterstützt wird.

3. Einrichtung zur Erzeugung einer Funktionsnanofaserschicht, die Partikel eines festen oder flüssigen Stoffes durch das elektrische Verspinnen der Polymerlösung oder -schmelze zwischen der Spinnelektrode (1) und der Sammelelektrode (2) aufweist, bei der die gebildeten Nanofasern zwischen der Spinnelektrode (1) und der Sammelelektrode (2) auf eine Unterlage gelagert werden, die die Oberfläche der Sammelelektrode (2) oder ein tragendes Material (8) ist, wobei hinter der Stelle und/oder in der Stelle der Lagerung der Nanofasern gegen die Unterlage mindestens ein Speicher (5) mit einer Ausgangsöffnung (51) zur Dosierung der Partikel des festen oder flüssigen Stoffes angeordnet ist, **dadurch gekennzeichnet, dass** die Ausgangsöffnung (51) des Speichers (5) mit der Gleitplatte (6) gekoppelt ist, die am der Unterlage zugewandten Ende eine scharfe Kante (61) aufweist, wobei die Gleitplatte (6) an die Hochspannungsquelle angeschlossen ist.

4. Einrichtung nach dem Anspruch 3, **dadurch gekennzeichnet, dass** die Gleitplatte (6) ans Ausgangsglied des Vibrators angeschlossen ist.

5. Einrichtung nach dem Anspruch 3 oder 4, **dadurch gekennzeichnet, dass** hinter der Stelle der Lagerung der eingetragenen Partikel eine Spinnelektrode (1, 12) gelagert ist.

## Revendications

1. Procédé de formation d'une couche nanofibreuse fonctionnelle comprenant des particules d'une substance solide ou liquide par l'électrofilage d'une solution ou d'un polymère fondu dans lequel les nanofibres formées sont déposées entre l'électrode de filage (1) et l'électrode collectrice (2) sur le substrat qui est la surface de l'électrode collectrice (2) ou le matériel de support (8), tandis que dans la couche ainsi formée immédiatement après sa formation dans le sens contre le substrat, on introduit entre ses nanofibres les particules de substance solide ou liquide qui sont placées dans l'espace entre les nanofibres, **caractérisé en ce que** l'introduction des particules dans la couche nanofibreuse est réalisée par l'action commune de la gravité, quand les particules sont guidées par la plaque coulissante inclinée (61) terminée par l'arête tranchante et par l'action de la haute tension entre le substrat et les particules qui en contact avec l'arête tranchante (61) de la plaque coulissante (6) obtiennent la charge électrique correspondante avec l'arête tranchante (61) chargée, tandis qu'en même temps il y a l'ionisation du milieu gazeux et le vent électrique qui est directionné à partir l'arête tranchante (61) de la plaque coulissante (6) ce qui facilite de transporter les particules introduites à la surface de l'électrode collectrice (2).

2. Procédé selon la revendication 1, **caractérisé en ce que** le mouvement des particules le long de la plaque coulissante inclinée (6) est soutenu par les vibrations de la plaque coulissante (6).

3. Dispositif pour former une couche nanofibreuse fonctionnelle comprenante des particules d'une substance solide ou liquide par électrofilage d'une solution ou du polymère fondu entre l'électrode de filage (1) et l'électrode de collectrice (2), dans lequel les nanofibres formées sont déposées entre l'électrode de filage (1) et l'électrode collectrice (2) sur le substrat qui est la surface de l'électrode collectrice (2) ou le matériel de support (8), tandis qu'après l'endroit et / ou le site de dépôt de nanofibres, au moins un conteneur (5) est prévu avec l'ouverture de sortie (51) pour distribuer des particules d'une substance solide ou liquide, **caractérisé en ce que** l'ouverture de sortie (51) du conteneur (5) est couplée à la plaque coulissante (6) équipé à l'extrémité tournée vers le substrat par l'arête tranchante (61), tandis que la plaque de glissement (6) est connectée à une source de la haute tension.

4. Dispositif selon la revendication 3, **caractérisé en ce que** la plaque coulissante (6) est reliée au membre de sortie du vibrateur.

5. Dispositif selon la revendication 3 ou 4, **caractérisé en ce qu'**une électrode de filage (1, 12) est disposée derrière le lieu de dépôt des particules introduites.
